

# United States Patent Office

3,410,768

Patented Nov. 12, 1968

1

3,410,768

**3,410,708**  
**METHOD OF PRODUCING CORROSION  
RESISTANT BERYLLIUM BODIES**

Louis J. Csontos, Parma, and Albert James Stonehouse, Lyndhurst, Ohio, assignors to The Brush Beryllium Company, Cleveland, Ohio, a corporation of Ohio  
No Drawing. Filed Sept. 8, 1964, Ser. No. 395,012  
14 Claims. (Cl. 204—37)

## ABSTRACT OF THE DISCLOSURE

A process for providing a corrosion resistant beryllium body by anodizing said body in an electrolytic bath containing sodium chromate and chromic acid at predetermined temperature and hydrogen ion concentration parameters, subsequently heat treating said body, and beryllium bodies and bodies having beryllium surfaces provided by said process having corrosion resistance under specified environments.

This invention relates generally to beryllium bodies having a corrosion resistant surface coating, and to a method for application of such a coating.

method for application of such a coating.

More specifically, the invention relates to anodized beryllium bodies having a corrosion resistant surface coating, and to a method for anodizing the surface of said bodies.

Beryllium metal has become well established for applications in inertial guidance systems, structural components for aircraft and aerospace use, and in other fields where its properties of lightness, high strength at elevated temperatures and its high strength to weight ratio are desirable characteristics.

However, commercially available beryllium is subject to corrosion by various environments, including high temperature air, tap water, deionized water, and salt spray. Various attempts have been made to provide corrosion resistant beryllium materials. Ceramic coatings have been applied to beryllium surfaces, and various methods of anodizing beryllium surfaces have been used, but all such

2

previously developed methods have failed to provide the desirable combination of properties obtained by the present method.

The present method provides corrosion resistant beryllium materials which greatly extend the application of beryllium in various fields, and was developed as a result of extensive investigation.

A primary object of the invention is to provide anodized corrosion resistant beryllium bodies.

A further object is to provide beryllium bodies resistant to corrosion in high temperature air, water, deionized water, and salt spray environments.

A still further object of the invention is to provide a method for applying a corrosion resistant coating to the beryllium surface of bodies.

Another object of the invention is to provide a method for anodizing the beryllium surfaces of bodies to render them corrosion resistant to high temperature, water, de-ionized water, and salt spray environments.

Other objects and advantages of the invention will become apparent from the following description.

The method comprises applying a protective surface coating to beryllium surfaces of bodies by passing an electric current to the beryllium surface connected as an anode, in a bath consisting essentially of water, sodium chromate in an amount of at least 0.4%, by weight, of the bath, and an amount of chromic acid sufficient to adjust the pH range of the bath from about 5.5 to about 7.5, preferably to about 7.0.

The concentration of the sodium chromate solution ranges generally from about 0.4% to about 10%, by weight of the bath, and preferably is used at a 5% weight concentration. The use of sodium chromate in excess of 10% does not appear to increase the effectiveness of the method or coating appreciably.

The bath should be free of hydrochloric and sulfuric acids, as their presence prevents formation of the desired protective coating.

The temperature of the bath must be maintained below about 130° F., since the coating applied above this temperature does not afford proper protective resistance. The temperature of the bath should be less than 130° F.

TABLE I.—PROCESS VARIABLES

| Example No.                                         | Voltage | Current Density, Amps/ft. <sup>2</sup> | Time (min.) | Wt. Conc. of Sodium Chromate, percent | pH  | Temperature of Bath in °F. | Hours Tested in 800° C. Dry Air | Physical Condition of Specimen After Test Exposure |
|-----------------------------------------------------|---------|----------------------------------------|-------------|---------------------------------------|-----|----------------------------|---------------------------------|----------------------------------------------------|
| <b>Effect of Anodizing Time:</b>                    |         |                                        |             |                                       |     |                            |                                 |                                                    |
| 1-----                                              | 12      | 170                                    | 10          | 5                                     | 7.0 | 75                         | 96                              | No attack or Failure.                              |
| 2-----                                              | 12      | 177                                    | 20          | 5                                     | 7.0 | 75                         | 96                              | Do.                                                |
| 3-----                                              | 12      | 166                                    | 30          | 5                                     | 7.0 | 75                         | 96                              | Do.                                                |
| 4-----                                              | 12      | 173                                    | 40          | 5                                     | 7.0 | 75                         | 96                              | Do.                                                |
| 5-----                                              | 12      | 162                                    | 50          | 5                                     | 7.0 | 75                         | 96                              | Do.                                                |
| 6-----                                              | 12      | 166                                    | 60          | 5                                     | 7.0 | 75                         | 96                              | Do.                                                |
| <b>Effect of Current Density:</b>                   |         |                                        |             |                                       |     |                            |                                 |                                                    |
| 7-----                                              | 10      | 49                                     | 60          | 5                                     | 7.0 | 75                         | 96                              | Do.                                                |
| 8-----                                              | 9       | 99                                     | 60          | 5                                     | 7.0 | 75                         | 96                              | Do.                                                |
| 9-----                                              | 12      | 150                                    | 60          | 5                                     | 7.0 | 75                         | 96                              | Do.                                                |
| 10-----                                             | 12      | 199                                    | 60          | 5                                     | 7.0 | 75                         | 96                              | Do.                                                |
| 11-----                                             | 12      | 298                                    | 60          | 5                                     | 7.0 | 75                         | 96                              | Do.                                                |
| <b>Effect of Solution Concentration:</b>            |         |                                        |             |                                       |     |                            |                                 |                                                    |
| 12-----                                             | 12      | 168                                    | 90          | 1                                     | 7.0 | 75                         | 161                             | Do.                                                |
| 13-----                                             | 12      | 160                                    | 60          | 2                                     | 7.0 | 75                         | 161                             | Do.                                                |
| 14-----                                             | 12      | 162                                    | 60          | 5                                     | 7.0 | 75                         | 161                             | Do.                                                |
| 15-----                                             | 9       | 160                                    | 60          | 10                                    | 7.0 | 75                         | 161                             | Do.                                                |
| <b>Effect of Increased Voltage:</b>                 |         |                                        |             |                                       |     |                            |                                 |                                                    |
| 16-----                                             | 18      | 162                                    | 10          | 1.5                                   | 7.0 | 75                         | 282                             | Do.                                                |
| 17-----                                             | 24      | 96                                     | 10          | 0.6                                   | 7.0 | 75                         | 282                             | Do.                                                |
| 18-----                                             | 24      | 166                                    | 10          | 1                                     | 7.0 | 75                         | 137                             | Do.                                                |
| 19-----                                             | 60      | 160                                    | 30          | 0.4                                   | 7.0 | 75                         | 96                              |                                                    |
|                                                     |         |                                        |             |                                       |     |                            |                                 |                                                    |
| <b>Hours tested in 1489° F. - 1,659° F. Dry Air</b> |         |                                        |             |                                       |     |                            |                                 |                                                    |
| <b>Effect of Temperature Variation:</b>             |         |                                        |             |                                       |     |                            |                                 |                                                    |
| 20-----                                             | 12      | 160                                    | 20          | 5                                     | 7.0 | 111                        | 203                             | Do.                                                |
| 21-----                                             | 12      | 160                                    | 60          | 5                                     | 7.0 | 176                        | 65                              | Failed, Corroded.                                  |
| 22-----                                             | 12      | 160                                    | 60          | 5                                     | 7.0 | 140                        | 65                              | Do.                                                |
| 23-----                                             | 12      | 160                                    | 60          | 5                                     | 7.0 | 75                         | 203                             | No Attack or Failure.                              |
| 24-----                                             | 12      | 160                                    | 60          | 5                                     | 7.0 | 129                        | 174                             | Do.                                                |

ranging from about 70° F. to about 110° F., and is preferably about 75° F.

For optimum resistance of the protective coating, the solution of sodium chromate should be prepared with distilled water and the pH adjusted with reagent grade chromic acid. The current density may vary from about 48 to about 300 amperes per square foot, and is preferably maintained at from about 150 to about 200 amperes per square foot. The current is applied for a period of time ranging from about 10 minutes to about 60 minutes.

Examples of beryllium bodies protectively coated by the method of the invention and exposed to high-temperature air environment are presented in the preceding Table I. In each example, a beryllium coupon 0.50" wide, 1.25" long and 0.1875" thick was protectively coated under the various processing conditions set forth in Table I.

Table II shows the effect of exposure to various testing environments of bodies protectively coated at the process conditions specified in the table.

TABLE II.<sup>1</sup>—EXPOSURE TESTS OF ANODIZED BERYLLIUM BODIES

| Example No. | Beryllium Body Size                              | Test Environment                           | Duration of Test | Condition of Bodies                                                                      |
|-------------|--------------------------------------------------|--------------------------------------------|------------------|------------------------------------------------------------------------------------------|
| 1           | 1" high x $\frac{1}{2}$ " Dia                    | 800° C. in 1% Moist Air                    | 1,749 Hrs.       | No attack or failure of anodic coating.                                                  |
| 2           | $\frac{1}{4}$ x $\frac{1}{2}$ x $\frac{3}{16}$ " | 850° C. in dry, CO <sub>2</sub> Free Air   | 185 Hrs.         | Do.                                                                                      |
| 3           | $\frac{1}{4}$ x $\frac{1}{2}$ x $\frac{3}{16}$ " | 900° C. in dry, CO <sub>2</sub> free air   | 137 Hrs.         | Do.                                                                                      |
| 4           | $\frac{1}{4}$ x $\frac{1}{2}$ x $\frac{3}{16}$ " | 1,000° C. in dry, CO <sub>2</sub> free air | 137 Hrs.         | Do.                                                                                      |
| 5           | $\frac{1}{4}$ x $\frac{1}{2}$ x $\frac{3}{16}$ " | 1,100° C. in dry, CO <sub>2</sub> free air | 113 Hrs.         | Do.                                                                                      |
| 6           | $\frac{1}{2}$ x $\frac{3}{8}$ x $\frac{1}{16}$ " | 700° C. in dry O <sub>2</sub>              | 100 Hrs.         | No attack or failure of anodic coating.<br>Wt. gain $\approx 0.1$ mg./cm. <sup>2</sup> . |
| 7           | $\frac{1}{2}$ x $\frac{3}{8}$ x $\frac{1}{16}$ " | 817° C. in dry O <sub>2</sub>              | 60 Hrs.          | No attack or failure of anodic coating.<br>Wt. gain = 0.33 mg./cm. <sup>2</sup> .        |
| 8           | $\frac{1}{2}$ x $\frac{1}{4}$ x $\frac{1}{16}$ " | 1,030° C. in dry O <sub>2</sub>            |                  | No attack or failure of anodic coating. Wt. gain = 0.58 mg./cm. <sup>2</sup> .           |
| 9           | $\frac{1}{8}$ " thick x $\frac{25}{16}$ " Dia    | 5% NaCl Salt Spray                         | 120 Hrs.         | No attack or failure of anodic coating.                                                  |
| 10          | 3" x 1" x $\frac{1}{16}$ "                       | 20% NaCl Salt Spray                        | 24 Hrs.          | Do.                                                                                      |
| 11          | 3" x 1" x $\frac{1}{16}$ "                       | 110° F. deionized water                    | 1,656 Hrs.       | Do.                                                                                      |
| 12          | 1" x $\frac{1}{4}$ " x $\frac{1}{8}$ "           | Tap Water                                  | 2,160 Hrs.       | Do.                                                                                      |
| 13          | 1" x $\frac{1}{4}$ " x $\frac{1}{8}$ "           | 0.1 N NaCl Soln.                           | 336 Hrs.         | Do.                                                                                      |

<sup>1</sup> All specimens included in Table II were anodized in a bath containing 5 weight percent sodium chromate with the pH adjusted to 7.0 with chromic acid at a temperature of 75° F., 12 volts and a current density of 160 amperes/ft.<sup>2</sup>.

It will be noted from Tables I and II that all the bodies with the exception of those protectively coated in Examples 21 and 22 of Table I at a bath temperature above 130° F., were completely protected from oxidation. No failure of the protective coating other than a slight change in color occurred, during test exposure of body specimens of all the other examples. Commercial beryllium when exposed to the same conditions normally oxidizes after 48 hours exposure to the extent that 25 to 50% of the test pieces will have been reduced to a fluffy powdered oxidation product.

A comparison exposure test of commercial beryllium specimens with the anodized bodies of Examples 6-8 inclusive, of Table II, showed that after exposure in one atmosphere of dry oxygen at 705° C. for 75 hours, 807° C. for 45 hours, and 1030° C. for 35 hours, the commercial specimens incurred a weight gain of 17.0, 63.0, and 37.0 mg./cm.<sup>2</sup>, respectively, a pronounced increase in weight compared to the weight gained by bodies of the examples even though the commercial specimens were tested for a shorter time at approximately the same temperatures. The examples thus illustrate the high corrosion resistance of the beryllium bodies, the surfaces of which are coated in accordance with the method of the invention.

The examples are presented as illustrative embodiments of the invention and include the preferred embodiments known at the time of preparation of the specification.

Although the method of applying the protective coating to beryllium bodies results in some dissolution of the

surface of the base metal, the overall dimensional change is less than 0.0001" per side, during application time of up to 60 minutes. The small dimensional change in the surface is the result of replacement of the removed beryllium by a protective coating, the volume of which is approximately equivalent to that of the removed metal.

Thus, the negligible dimensional change which occurs in the surface during application of the protective coating is unexpected, as beryllium oxide is known to occupy a larger volume than the amount of beryllium metal stoichiometrically required to produce a given quantity of oxide. The final surface of the protectively coated body is identical in surface pattern with the original body surface, as the degree of polish, machining marks, and blemishes are faithfully reproduced.

18 The coatings applied by the method of the invention  
are quite dense and relatively thick. Generally, the thick-  
ness of the coating varies from 0.1-2.4 mils, but prefer-  
ably is about 0.5 mils, dependent upon the control of the  
20 process conditions.

## PERIODICITY TESTS

The protective coating applied is believed to be a form of hydrated beryllium oxide as it is nearly amorphous in the initially deposited form, as indicated by X-ray analysis. When heated at elevated temperature for a sufficient time, the initial coating is converted to normal crystalline beryllium oxide, as evidenced by X-ray diffraction analysis. Temperatures of about 800° C. may be employed for effecting conversion to the crystalline state.

55 Having thus described our invention, we claim:

1. The method of applying a protective surface coating to a beryllium surface of a body, comprising: passing an electric current to the surface with the surface connected as an anode and immersed in a bath consisting essentially of water, sodium chromate in an amount at least 0.4%, by weight, of the bath, and an amount of chromic acid sufficient to adjust the pH of the bath into a range from about 5.5 to about 7.5, the temperature of the said bath being below about 130° F.

65 2. The method according to claim 1 wherein the sodium chromate ranges from about 0.4% to about 10%, by weight, of the bath, and a sufficient amount of chromic acid is present in each concentration of sodium chromate to maintain the pH of the bath from about 5.5 to about 7.5.

3. The method according to claim 1 wherein the electric current density is from about 48 to about 300 amperes per square foot.

75 per square foot.

4. The method according to claim 1 wherein the electric current is applied from about 10 minutes to about 60 minutes.

5. The method according to claim 1 wherein the water is distilled water and the pH is adjusted by reagent grade chromic acid.

6. The method according to claim 1 wherein the bath temperature ranges from 70° F. to about 110° F.

7. The method according to claim 1 wherein the body consists essentially of beryllium.

8. The method according to claim 1 wherein, after application, the coating is heated to a temperature sufficient to convert the coating to crystalline beryllium oxide.

9. The method according to claim 8 wherein said temperature is about 800° F.

10. A method of applying a protective surface coating to beryllium, comprising: passing an electric current having a density of from about 150 to about 200 amperes per square foot to a body having a beryllium surface connected as anode and immersed in a bath consisting essentially of water, about 5% sodium chromate, by weight of said bath, and an amount of chromic acid sufficient to adjust the pH of the bath to about 7.0, the temperature of said bath being about 75° F.

11. The method according to claim 10 wherein the water is distilled water and the pH is adjusted by reagent grade chromic acid.

12. A bath for the electrolytic production of protective corrosion-resistant coatings on beryllium surfaces, consisting essentially of water, sodium chromate in a concentration ranging from about 0.4% to about 10%, by

10

15

20

25

weight of the bath, and adjusted by an addition of chromic acid to a pH of about 7.0, said bath being free of hydrochloric and sulfuric acids, respectively.

13. A bath according to claim 12 wherein the concentration of the sodium chromate is approximately 5%.

14. A bath according to claim 12 wherein the water is distilled water, and the chromic acid is reagent grade.

#### References Cited

##### UNITED STATES PATENTS

|           |         |         |       |          |
|-----------|---------|---------|-------|----------|
| 2,606,866 | 8/1952  | Neish   | ----- | 204—56   |
| 2,871,425 | 1/1959  | Burnham | ----- | 204—56 X |
| 3,276,974 | 10/1966 | Tyson   | ----- | 204—56 X |

##### OTHER REFERENCES

Levin, M. L.: "The Formation of Crystalline Anodic Oxide Films on Beryllium"—Transactions of The Faraday Society, vol. 54, pp. 935—940, 1958.

Whitby, L. et al.: "Chromic Acid Anodizing of Beryllium"—Proceedings of The American Electroplater's Society, col. 48, pp. 106—108, 1961.

Missel, Leo: "Chromic Acid Anodizing of Beryllium"—Proc. of The American Electroplater's Society, vol. 48, pp. 109—111, 1961.

HOWARD S. WILLIAMS, *Primary Examiner.*

G. KAPLAN, *Assistant Examiner.*